

Jan. 23, 1923.

1,442,840

J. H. WRIGLEY,  
FINISHING FABRICS.  
FILED FEB. 25, 1920.



Inventor  
J. H. Wrigley  
by Wright, Brown, Dimby & May  
Attorneys

## UNITED STATES PATENT OFFICE.

JOHN HERBERT WRIGLEY, OF MANCHESTER, ENGLAND, ASSIGNOR TO BRADFORD  
DYERS' ASSOCIATION LIMITED, OF BRADFORD, ENGLAND.

## FINISHING FABRICS.

Application filed February 25, 1920. Serial No. 361,229.

*To all whom it may concern:*

Be it known that I, JOHN HERBERT WRIGLEY, a subject of the King of Great Britain, and resident of 4 Darley Road, 5 Whalley Range, Manchester, in the county of Lancaster, have invented a certain new and useful Improvement in Finishing Fabrics, of which the following description, together with the accompanying sheet of 10 drawings, is a specification.

In certain parts of the process of treating fabrics in order to carry out the finishing or preparing of said fabrics for the market or for use, they are subjected to the actions 15 of devices which apply pressure to them intermittently, such as in apparatus known as a beetling machine. In varied processes of this character results are obtained which give the fabrics certain lustrous effects, and 20 to enhance these lustrous effects and give a more distinctive appearance to the fabrics thus treated by the application of means or devices of a novel and original character, is the object of my present invention.

25 In the varied processes in which fabrics are treated by being intermittently subjected to the actions of pressure, said pressure has been applied by falling beetles in a beetling machine. In these machines or 30 apparatus the resultant effects are of a distinctive character but are accompanied by defects (such as what are known in the trade as "watered" or moiré effects) which are undesirable.

35 By means of my invention I am able to give a finish to the fabrics in a uniform degree throughout so that the whole of the surfaces of said fabrics present a better and more desirable appearance.

40 According to my invention I produce a roll consisting of alternate layers of fabric and of yielding material such as rubber, preferably by winding simultaneously onto a roller a length or piece of fabric and a 45 corresponding length of rubber sheet or web. Pressure is applied to the multiplicity of alternate layers of fabric and rubber thus produced preferably intermittently by the ordinary beetling process and whilst the roll 50 is still on the roller.

In order to be enabled to more clearly describe my invention I do so by reference to the accompanying sheet of drawings

which shows the preferred manner of carrying out my invention, and in which:—

55 Fig. 1 is intended to show a fabric as being wound upon the roller of a beetling machine simultaneously with the winding thereon of an elastic fabric, which intervenes between the coils of the other fabric. 60

Fig. 2 is a perspective view of a fabric drawn to a greatly enlarged scale in order to show the manner in which my improved devices act.

When my invention is put into practice 65 the pressing devices act evenly over the whole of the irregular surfaces of the fabrics being treated, whereas when fabrics are compressed under the ordinary conditions only those parts of the fibres which extend 70 most prominently from their surfaces are acted upon. In accordance with my invention I insert a yielding substance *f* between the pressing surfaces of the beetles *a* and between layers with the fabric *c* so that 75 when the beetles descend the layers *f* are pressed upon the fabric *c* in a yielding manner.

The yielding substance *f* which I have found to act efficiently is sheet india rubber 80 or an india rubber covered fabric.

I wind the rubber or like substance *f* onto the roller *g* simultaneously with the fabric *c* to be treated. When the winding of the compound or duplex coils is completed, 85 rotation of the coil is continued and the beetles *a* are brought into operation in the ordinary manner for such a period as is found necessary to secure the results aimed at. For a material such as fine cotton taf- 90 fettas with a roll about eighteen inches diameter with beetles about four inches wide by three inches thick each giving sixty blows per minute, I find excellent results are produced if the beetling is continued for about 95 ten minutes. Then the fabric and rubber are wound off onto another roller so as to reverse the ends in the usual manner after which they are again treated for about ten minutes to finish the process. I obtain by 100 my invention carried out in this manner a uniform finish such as I have not been able to obtain previously. Presumably by reason of the beetles *a* acting upon the fabric *c* through the medium of the rubber *f* which 105 rubber *f* in addition to resting upon the

more prominent fibres *d* will be caused to bend and extend over and down upon same as shown at *e* by Fig. 2, thus as the pressure is applied to the yielding substance *f* it rubs or moves down over the fibres *d* as shown at *e* while on the removal of said pressure it returns and again exerts its rubbing action over said fibres.

Such being the nature and object of my 10 said invention, what I claim is:—

1. In the finishing of fabrics, intermittently applying pressure to a roll consisting of a multiplicity of alternate layers of yielding material and fabric.
- 15 2. In the finishing of fabrics, simultaneously winding on to a roller, a fabric and a yielding material to produce a multiplicity

ity of alternate layers and subsequently applying pressure thereto for the purpose described.

3. In the finishing of fabrics, simultaneously winding on to a roller a fabric and a sheet of rubber to produce a multiplicity of alternate layers of fabric and rubber, and subsequently applying intermittent pressure 25 thereto.

4. In the finishing of fabrics, simultaneously winding on to a roller a fabric and a yielding material to produce a multiplicity of alternate layers of fabric and yielding 30 material, and apply pressure thereto by beetling.

JOHN HERBERT WRIGLEY.